

July 6, 1937.

J. F. FERM ET AL.

2,085,963

## METHOD OF MAKING A DEFORMED BAR

Filed July 12, 1935

2 Sheets-Sheet 1

Fig. 1.



Fig. 1A.



Fig. 2.



Fig. 3.



Fig. 4.



25 74



INVENTORS  
John F. Ferm & Fred S. High  
by his attorneys  
Byrnes, Stebbins & Blenko

July 6, 1937.

J. F. FERM ET AL

2,085,963

METHOD OF MAKING A DEFORMED BAR

Filed July 12, 1935

2 Sheets-Sheet 2



*Fig. 8.* *Fig. 9.* *Fig. 10.* *Fig. 11.*



20 INVENTORS  
John F. Ferm & Fred S. High  
by their attorneys  
Byrnes, Stetinius & Blanko

## UNITED STATES PATENT OFFICE

2,085,963

## METHOD OF MAKING A DEFORMED BAR

John F. Ferm and Fred S. High, Midland, Pa.,  
assignors to Pittsburgh Crucible Steel Company, Pittsburgh, Pa., a corporation of Pennsylvania

Application July 12, 1935, Serial No. 30,998

## 10 Claims.

(Cl. 80—60)

Our invention relates to a deformed bar such as a forging blank and the method by which it is manufactured.

Forging blanks have been made by die rolling for a considerable period. The methods which have been employed in the past, however, are objectionable for a number of reasons. The principal desideratum of a forging blank is that it shall lie flat in the forging dies, but this result has not been satisfactorily produced by the methods previously practiced.

In U. S. Patent 1,923,017, granted to Witherow et al., there is disclosed a method of making forging blanks by subjecting a leader to rolling in two separate passes, the leader being deformed in the first pass to provide spaced masses of metal, and flattened in the second pass. The two-pass method was subsequently improved and, as a result, a one-pass method disclosed in U. S. Patent 1,998,970, granted to Thomas N. Sloan, came into use. Sloan employs die rolls having matrix grooves of varying width and depth, and forms a forging blank by a single passage of a leader therethrough to fill, but not over-fill, the matrix grooves. The pass is substantially closed, that is, it has side walls which prevent excessive lateral flow of the metal and actually exert a shaping effect on the leader.

We have improved on the methods of the prior art in that we are able to roll a forging blank in one passage between deforming rolls defining an open pass, that is, without side walls, which compress and elongate a leader in spaced portions, without substantial lateral spreading of the metal thereof. As a result, we are able to produce a forging blank having spaced masses of metal connected by reduced portions, the blank having substantially flat sides so that it lies squarely in the forging dies and is very easy to manipulate therein. The use of an open pass considerably simplifies the design thereof and reduces roll wear.

In accordance with our invention, we utilize a leader having concave sides. The concavity of the sides may be produced by well known means in the latter stages of rolling the leader. When the leader with concave sides is passed through deforming rolls defining an open pass, the leader is heavily reduced and considerably elongated in spaced portions thereof, and is only slightly reduced and elongated in the remaining portions thereof. In neither case is there any substantial lateral spreading of the leader. There is a slight spreading only in the portions which are more heavily reduced, but this only has the effect of

squeezing out the original concavity of the sides of the leader in such portions and the resulting blank has substantially flat sides.

For a complete understanding of the invention, reference is made to the accompanying drawings illustrating a preferred practice of the method and a preferred form of the product, although it is to be understood that changes in both may be made within the scope of our broader claims. In the drawings—

Figure 1 is a side elevation of the leader which we employ;

Figure 1a is an end elevation thereof;

Figure 2 is a diagrammatic side elevation, partly in section, of the roll pass by which the leader 15 is formed into a string of forging blanks;

Figure 3 is a section through one of the rolls along the line III—III of Figure 2.

Figure 4 is a sectional view along the line IV—IV of Figure 2;

Figure 5 is a sectional view similar to Figure 3 showing a modified form of roll pass;

Figure 6 is a side elevation of a forging blank produced in accordance with our invention, after it has been sheared from the string with which it was rolled;

Figure 7 is a plan view thereof;

Figure 8 is an end elevation of the blank;

Figure 9 is a sectional view along the line IX—IX of Figure 6;

Figure 10 is a sectional view along the line X—X of Figure 6; and

Figure 11 is a sectional view along the line XI—XI of Figure 6.

Referring now in detail to the drawings, a leader 10 which is simply a relatively long billet, has a generally rectangular cross section, the top 11 and the bottom 12 thereof being substantially flat. The sides 13 of the leader, however, are concave as shown (somewhat exaggerated) in Figure 1a. The corner edges of the leader are rounded in accordance with the usual practice. The leader is formed into a string of forging blanks by passing it between deforming rolls 14, with its greater cross sectional dimension perpendicular to the axes of the rolls.

The rolls 14 have spaced protuberances or projections 15, 16 and 17 thereon, effective to squash down or compress and elongate spaced portions of the leader. The exact conformation and disposition of the projections or protuberances depend, of course, upon the nature of the blank to be produced. Merely by way of example, we have illustrated a blank 18 adapted to be forced into a crank shaft. The blank 18 comprises reduced

5

10

20

25

30

35

40

45

50

55

- end portions 19, one of which (as shown at the left in Figure 6), is extended to form a tong-hold 20, enlarged end portions 21, reduced middle portions 22 and a slightly reduced middle portion 23.
- 5 As shown in Figures 8 and 10, the portions 19, 20 and 22 of the blank have curved upper and lower surfaces and relatively flat sides. The portions 21 and 23 of the blank, as shown in Figures 9 and 11, are relatively rectangular in section.
- 10 From a comparison of Figures 2 and 6, it will be apparent that the projections 15 form the sections 19 and 20 of adjacent blanks in a string. Likewise, projections 16 and 17 form the spaced portions 22 of the blanks. These projections of 15 the rolls are curved as shown at 15a in Figure 4, to produce the desired contour of the portions 19, 20 and 22. The portions of the rolls between the projections 15 and 16 and 15 and 17 indicated at 24, are flat except for the fillets 25 (Figure 3) necessary to produce the desired curvature at the corners of the rectangular portions of the blanks. The portions of the roll between the projections 16 and 17, indicated at 25a, form the central enlarged portion 23 of the blanks, and 25 are similar to the roll portions 24 except that they have a slightly larger diameter.

The rolls 14 are provided adjacent the projections 15, 16 and 17 with collars 26. The collars 26 serve merely as guides for the tools employed 30 to finish the portions of the roll engaging the leader. The collars 26 do not constitute side walls of a matrix groove in the rolls. There is, in fact, no matrix groove but only a plurality of alternately flat and rounded portions of different 35 diameter. It will be observed that the collars 26 are connected to the fillets 25 by sloping wall portions 27 in the form of roll shown in Figure 3. The collars are actually spaced axially of the rolls from the working portion thereof in the 40 form of roll shown in Figure 5. The curved portions 15a of the roll faces feather off into the collars 26 by long radius fillets 28. Thus, in no portion of the roll is there any confinement of the leader against lateral spreading. The slight 45 curvature of the fillets 25 and 28, of course, does not preclude such lateral spreading. Rolling of the leader in accordance with our invention is effected without any substantial confinement thereof against lateral spreading or extrusion.

50 In spite of this fact, we are able to produce substantially flat sided blanks by starting with a billet having concave sides.

It will be observed that the rolls 14 are spaced a considerable distance apart. Even the collars 55 26, which take no part in the actual reduction of the leader, are separated by a considerable distance, amounting, in a specific case, to  $1\frac{1}{8}$ ". The pass between the rolls 14 is thus open at all portions around the roll peripheries. The use 60 of an open pass without side walls has a particular advantage in that the design of the roll pass is thereby greatly simplified and wear on the rolls materially reduced.

By reference to Figure 7, it will be observed 65 that the sides of the finished blank, indicated at 13', are substantially flat considered overall. There is, of course, a slight deviation from a true plane, but this is not such as to prevent the blanks from lying flat in the dies, thus facilitating manipulation thereof as the forging proceeds. 70 It will be apparent from what has been said, and from the showing of Figure 7, that in those portions of the blank, 19, 20 and 22, which are heavily reduced, the originally concaved side walls of the leader are spread out slightly as the 75

result of the crushing down of the leader so that in the finished product they have a very slight convexity. In those portions of the blank which are only slightly reduced, 21 and 23, the original concavity of the sides remains substantially unaltered. The finished blank, however, has a plurality of enlarged portions connected by portions of reduced cross section, the blank being substantially flat along its sides, the greatest variations in size being in the dimension measured along 10 the sides. The corner edges of the blank are substantially straight when viewed in plan.

The advantages of our invention over the two-pass method or the one-pass method using die rolls having matrix grooves with side walls, will 15 be readily apparent. All the difficulties encountered because of rolling in two passes are avoided. At the same time, our die rolls without side walls are much easier to make than die rolls having side walls exerting a shaping action on the leader. 20 The wear on the rolls is also considerably less because the only action thereof is a substantially direct compression of the leader without any lateral extrusion thereof to fill in the space defined by the side walls of die rolls having matrix 25 grooves provided therewith.

Although we have illustrated and described herein but one preferred practice of our method and one embodiment of the article resulting therefrom, it will be apparent that many changes 30 in both may be made without departing from the spirit of the invention or the scope of our appended claims. The invention is applicable generally to the rolling of deformed bars and its advantages are not confined to the manufacture 35 of forging blanks, the latter being specifically disclosed herein merely by way of example.

We claim:

1. In a method of making a forging blank having substantially flat sides so as to lie flat in a 40 forging die, and spaced masses separated by predetermined distances but connected by intermediate portions of sectional area less than that of said masses, the steps including forming a leader having a generally rectangular section, two opposite concave surfaces, and two opposite substantially flat surfaces, passing the leader between rolls with the flat surfaces substantially parallel to the roll axes, to form said masses and elongate said intermediate portions by so crushing the 45 leader without substantial confinement thereof against lateral spreading, that the portions suffering greatest deformation are bulged substantially into the plane determined by the edges of the originally concave sides. 55

2. In a method of making a forging blank having substantially flat sides so as to lie flat in a forging die, and spaced masses connected by intermediate portions of less sectional area than said masses, the steps including forming a generally rectangular leader with two opposite concave sides, passing the leader between rolls effective to compress the remaining sides of the leader without substantially confining the concave sides, and form said masses and portions, the portions 60 suffering greatest deformation being bulged substantially into the plane determined by the edges of the originally concave sides. 65

3. In a method of making a forging blank having substantially flat sides so as to lie flat in a 70 forging die and spaced masses connected by intermediate portions of less sectional area than said masses, the steps including passing a leader having concave opposite sides between rolls effective to compress the leader progressively in a plane 75

substantially perpendicular to said sides without substantial confinement against lateral flow, and so deforming the bar that the portions suffering greatest deformation are bulged substantially into 5 the plane determined by the edges of said originally concave sides.

4. In a method of making a forging blank capable of lying flat in a die, the steps including subjecting a leader with concave sides to a material reduction in thickness between its top and 10 its bottom, in longitudinally spaced portions only.

5. In a method of making a forging blank that will lie flat in a die, the steps including subjecting a leader to material reduction of its thickness between its top and bottom, in longitudinally spaced 15 portions only, and limiting lateral extrusion of the leader by concaving its sides before said reduction.

6. In a method of making a forging blank capable of lying flat in a forging die, the steps 20 including forming a leader having concave sides, and subjecting the leader to material reduction in the thickness between its top and bottom, in longitudinally spaced portions only, by rolling in a pass open at the sides.

25 7. In a method of making a forging blank that will lie flat in a forging die, the steps including providing a leader with concave sides, subjecting the leader to a single rolling pass effective to materially reduce the top-to-bottom dimension of 30 longitudinally spaced portions only of the leader without confinement thereof against lateral spreading.

8. In a method of making a forging blank that will lie flat in a forging die, the steps including rolling a leader with concave sides, positioning the leader with said sides substantially vertical, passing it between horizontal rolls to reduce slightly 5 the vertical dimension of the leader, and reducing and elongating longitudinally spaced portions thereof only, to a greater extent, without substantially confining the leader against lateral flow.

9. In a method of rolling a forging blank 10 capable of lying flat in a forging die and having one substantially uniform cross sectional dimension, the other cross sectional dimension varying along the length of the bar, the steps including passing a leader between rolls having circumferentially spaced protuberances effective to reduce materially the height of longitudinal spaced portions only of the leader, and limiting the maximum widening of the leader as a result of the 15 rolling, by imparting concavity to the sides of the 20 leader before subjecting it to rolling.

10. In a method of making a forging blank that will lie flat in a forging die, the steps including forming a leader having concave sides and a substantially flat top and bottom, and passing the 25 leader between rolls having circumferentially spaced protuberances effective to reduce materially the height of longitudinally spaced portions only of the leader without confining said sides against lateral flow.

JOHN F. FERM.  
FRED S. HIGH.